

# UNITED STATES PATENT OFFICE.

MYRTIL KAHN AND ANTON OSSENBECK, OF ELBERFELD, GERMANY, ASSIGNEES TO  
FARBENFABRIKEN VORM. FRIEDR. BAYER & CO., OF ELBERFELD, GERMANY, A  
CORPORATION OF GERMANY.

## BLACK MORDANT MONOAZO DYESTUFF.

1,078,925.

No Drawing.

Specification of Letters Patent.

Patented Nov. 18, 1913.

Application filed December 6, 1912. Serial No. 735,262.

To all whom it may concern:

Be it known that we, MYRTIL KAHN and ANTON OSSENBECK, citizens of the German Empire, residing at Elberfeld, Germany, have invented new and useful Improvements 5 in Black Mordant Monoazo Dyestuffs, of which the following is a specification.

We have found that new and valuable mordant monoazo dyestuffs are obtained by 10 combining diazo compounds of ortho-amino-phenol-sulfonic acids with acidyl-1-amino-7-naphthols. The new products thus produced are mordant dyestuffs. They dye wool from acid baths in violet shades, 15 which by aftertreatment with chromates change into bluish-black to greenish-black shades fast to light and fulling. They also dye wool in one bath in the presence of a chrome mordant. They are after being 20 dried and pulverized in the shape of their alkaline salts dark powders soluble in hot water violet; yielding upon treatment with stannous chlorid and hydrochloric acid an ortho-aminophenol-sulfonic acid and 1.8-diamino-7-naphthol.

In order to illustrate the new process more fully the following example is given, the parts being by weight:—22.4 parts of 4-chloro-2-aminophenol-6-sulfonic acid are 25 azotized with 7 parts of sodium nitrite. The diazo compound is then added to a solution containing an excess of sodium carbonate of 21 parts of acetyl-1-amino-7-naphthol in the calculated quantity of dilute 30 caustic soda lye. The production of the dyestuff is soon finished. It is filtered off, pressed and dried. It has most probably the formula:



and is after being dried and pulverized in the shape of its sodium salt a brownish-black

powder soluble in hot water with a violet 50 coloration. It dyes wool from an acid bath in violet shades which on being chromed change into a blue-black fast to light and fulling. Upon treatment with stannous chlorid and hydrochloric acid it is split 55 up into 2-amino-1-phenol-4-chloro-6-sulfonic acid and 1.8-diamino-7-naphthol. 2-amino-phenol-4-sulfonic acid itself or other derivatives of this acid *e. g.* ortho-amino-para-cresol-sulfonic acid or 6-chloro-2-amino-phenol-4-sulfonic acid may be used. Other acidyl-1-amino-7-naphthols such as the benzoyl compound may be used.

We claim:

1. The herein described new mordant 65 mono-azo dyestuffs of the following graphically represented structure  $R-N=N-R'$  where R is the radical of an ortho-phenol-sulfonic acid and R' the radical of an acidyl-1-amino-7-naphthol, which are after being 70 dried and pulverized in the shape of their alkaline salts dark powders soluble in hot water generally with a violet coloration; yielding upon reduction with stannous chlorid and hydrochloric acid a 2-amino-75 phenol-sulfonic acid and 1.8-diamino-7-naphthol; dyeing wool in violet shades which after being chromed change into fast bluish-black to greenish-black shades and dyeing wool in one bath in the presence of 80 a chrome mordant, substantially as described.

2. The herein described new azo dyestuff having most probably the formula:



which is after being dried and pulverized 95 in the shape of its sodium salt a brownish-black powder soluble in hot water with a violet coloration; yielding upon reduction

with stannous chlorid and hydrochloric acid  
2-amino-1-phenol-4-chloro-6-sulfonic acid  
and 1,8-diamino-7-naphthol; dyeing wool in  
violet shades which after being chromed  
5 change into a blue-black fast to light and  
fulling, substantially as described.

In testimony whereof we have hereunto

set our hands in the presence of two sub-  
scribing witnesses.

MYRTIL KAHN. [L. S.]  
ANTON OSSENBECK. [L. S.]

Witnesses:

HELEN NUFER,  
ALBERT NUFER.